

## 1

2,845,376

## METHOD OF COATING METAL SURFACES WITH PHOSPHATE

Montagu Hyams, London, England, assignor, by direct and mesne assignments, to Neilson Chemical Company, Detroit, Mich., a copartnership

No Drawing. Application June 9, 1953  
Serial No. 360,597

5 Claims. (Cl. 148—6.15)

This invention relates to the surface treatment of metal by the chemical action thereon of a water-miscible surface treating medium.

The chemical surface treatment of metal is normally carried out by contacting the surface of metal with a large volume of treating liquid, applied by immersion or by spraying. This involves the disadvantage, especially in cleaning processes, that a large volume of liquid to be used in subsequent treatments becomes contaminated during the treating process. Moreover, especially in coating processes, supersaturation or desired pH change at the liquid/metal interface takes place but slowly due to the washing action of the ever changing liquid at the interface. Another disadvantage of this type of treatment is that, where the treating liquid is to be applied hot, a large volume of liquid must be maintained in heated condition.

These disadvantages may be overcome by applying the surface treating medium to the metal surface as a film and allowing the film to remain on the metal surface until the desired degree of treating action has been achieved. Such film processes as carried out hitherto have had limited application, however, and for many applications have not been at all satisfactory. It has normally been found necessary to operate at room temperature or, if elevated temperatures are to be used, to contact the metal only for short periods and with dilute solutions, to prevent premature drying of the film. The use of dilute solutions has meant insufficiency of active material at the metal surface and of such short heating periods that the process usually is incomplete. In such processes the film quickly dries, the chemical action ceases and there is left upon the metal surface a difficultly removable or washable residue. If the surface undergoing treatment is of ferrous metal, there is very great tendency for the drying surface to oxidise and rust under the influence of the atmosphere.

An object of the present invention is to provide a process for the surface treatment of metal by the chemical action thereon of a water-miscible surface treating medium, in which process the advantages of film application as set out above are fully obtained, and in which high concentrations of liquid may be applied at elevated temperature until the treating action has reached the desired degree of completion without the attendant disadvantages normally associated with film type processes as set out above.

According to the present invention, a process of treating the surface of metal by the chemical action thereon of a water-miscible surface treating medium comprises providing upon said surface a film of said medium and contacting the film so provided with steam having a temperature in excess of 180° F.

The surface treating process may be a coating process wherein the metal surface is provided with an adherent non-metallic coating, such as an insoluble metal phosphate coating. In such processes, the presence of a polyvinyl methyl ether or of a polyoxyethyleneoxypropylene

## 2

glycol or ether thereof in the coating medium may facilitate coating formation.

The said film may be applied to the surface undergoing treatment by immersing the surface in, or by flowing or spraying onto said surface, a liquid or powdered or paste-like surface treating medium. Application of steam to the film may involve immersing the film in a bath of steam or directing steam in spray or jet form onto the film, or both.

10 According to one feature of the invention, the metal surface bearing the film of surface treating medium, especially a coating liquid, is immersed in a bath of steam, as for example in a conventional bottle sterilising plant, until the treating action, for example the coating process, is substantially complete.

According to another feature of the invention, the film of surface treating medium is sprayed with steam continuously or intermittently, until the treatment is substantially complete. When the steam is sprayed intermittently, it is preferred to renew the film after at least one other than the last spraying period.

20 The invention finds particularly useful application in the phosphate coating of metals, especially of ferrous metals, and will be illustrated with this field of application in mind.

25 The following examples illustrate the invention.

## Example I

30 A coating solution was prepared from 175 parts by weight of zinc dihydrogen phosphate dihydrate, 30 parts by weight of 42° Bé. nitric acid, 1.5 parts by weight of copper carbonate and 295 parts by weight of water. Iron wire to be drawn was uncoiled from a roll and given a thin film of the cold coating solution by passing through 35 rollers provided with a film of the coating material. The wire issuing from the rollers was passed through a narrow tube which was thermally lagged and in which steam at substantially atmospheric pressure was slowly circulated counter-current to the direction of travel of 40 the wire. The rate of travel of the wire through the steam-filled tube was such that the residence time of a given section of the wire in the tube was 30 secs. The treated wire emerging from the steam-filled tube was passed through a water spray rinse zone and was found to have an excellent coating of zinc phosphate for facilitating the subsequent drawing process.

## Example II

45 A number of rusty steel bolts were loaded into a perforated barrel rotatable upon its horizontal axis. The barrel was immersed in a cold solution formed by dissolving one part by volume of 75% orthophosphoric acid in two parts by volume of water. The barrel was immersed in the solution for 5–10 seconds and then removed and allowed to drain. The barrel was then rotated about its horizontal axis in a loosely enclosing sheath while steam from a 20 p. s. i. source was continuously led into the inside of the rotating barrel and escaped through the perforations and out through the 50 space between the wall of the barrel and the enclosing sheath. After three minutes of such treatment the bolts had become coated with a uniform coating of iron phosphate and were free from rust.

## Example III

60 A steel panel, somewhat imperfectly freed from rust and grease, was treated in a conventional spray plant by means of a decimolar solution of sodium dihydrogen orthophosphate sprayed onto the panel at a temperature of 150° F., the solution also containing a trace of wetting agent. After two minutes spraying the panel was imperfectly coated with iron phosphate. In another process-

ing run, the panel was treated in similar fashion except that after every 20 secs. of processing the sprays of liquid were cut off and the work was sprayed with steam from a 20 p. s. i. source. After two minutes operation in all, the panel was coated uniformly over its whole surface, the steam treatment having activated the metal surface, especially the more difficultly coated portions of the surface.

*Example IV*

A refrigerator cabinet of ferrous metal was supported horizontally about its central longitudinal axis two-thirds immersed in a conventional cold phosphating solution maintained at around room temperature and pH of 2.25 and containing, in g. p. l. of bath, 19.5 Zn, 23.2 P<sub>2</sub>O<sub>5</sub>, 19.3 Na and 69.8 NO<sub>3</sub>. The solution also contained 2% by weight of polyvinyl methyl ether. The refrigerator cabinet was slowly rotated about its horizontal axis while supported in the processing solution, and near the top of its travel out of the solution the cabinet was subjected to the action of steam sprayed onto it from a 20 p. s. i. source. After five minutes of such treatment the processing bath had not increased in temperature by more than 2-3° F. and the cabinet was covered with a fine uniform coating of zinc phosphate of much finer grain and uniformity than when the mild steam heating was not applied. It is believed that this was due partly to the heat facilitating the seeding out of tertiary zinc phosphate, and to the polyvinyl methyl ether which was reversibly precipitated by the heating action facilitating the precipitation of the seeded zinc phosphate and preventing clogging of the surface with too rapidly precipitated and loosely adherent zinc tertiary phosphate. Instead of polyvinyl methyl ether, a polyoxypropyleneoxyethylene glycol of around 40° C. flocculation temperature may be used.

*Example V*

Food cans of steel are brushed with a coating solution prepared as described in Example I. The coated cans are led suspended from a travelling chain in zig zag manner through the chamber of a conventional bottle sterilising machine maintained at a temperature in the chamber of around 185° F. Upon emerging from the machine after having travelled therein for two minutes they have an excellent adherent surface coating of insoluble metal phosphate.

I claim:

1. Process of providing upon the surface of metal an adherent coating of insoluble metal phosphate through the chemical action upon said surface of an acidic, water-miscible phosphatising liquid, which comprises providing upon said surface a film of said liquid and subsequently, while said film is still in the liquid state, spraying steam having a temperature in excess of 180° F. in substantially continuous manner upon the film so provided until the desired degree of coating has been attained, said film being replenished with coating liquid at least once during the period in which steam is applied thereto.

2. Process of providing upon the surface of metal an

adherent coating of insoluble metal phosphate through the chemical action upon said surface of an acidic, water-miscible phosphatising liquid, which comprises providing upon said surface a film of said liquid and subsequently, while said film is still in the liquid state, spraying steam having a temperature in excess of 180° F. intermittently upon the film so provided until the desired degree of coating has been attained, said film being replenished with coating liquid after at least one period of spraying with steam other than the last such period.

3. Process of providing upon the surface of metal an adherent coating of insoluble metal phosphate which comprises successively immersing the surface in and withdrawing the surface from, a bath of phosphatising solution a plurality of times and subsequently, while said film is still in the liquid state, spraying steam having a temperature in excess of 180° F. upon the metal surface between successive immersion periods.

4. Process of providing upon the surface of metal an adherent coating of insoluble metal phosphate which comprises successively immersing the surface in and withdrawing the surface from, a bath of phosphatising solution a plurality of times and subsequently, while said film is still in the liquid state, spraying steam having a temperature in excess of 180° F. upon the metal surface between successive immersion periods, said phosphatising solution containing a compound which is precipitated upon heating, and redissolved upon cooling, the solution and is selected from the group consisting of polyvinyl methyl ethers, polyoxyethyleneoxypropylene glycols and polyoxyethyleneoxypropylene glycol ethers.

5. Process of providing upon the surface of metal an adherent coating of insoluble metal phosphate which comprises applying a phosphatising liquid to a metal surface to form a film thereon, and subsequently, while said film is still in the liquid state, applying steam to said film to complete the phosphate coating action.

References Cited in the file of this patent

UNITED STATES PATENTS

|              |              |       |               |
|--------------|--------------|-------|---------------|
| 753,610      | McDowell     | ----- | Mar. 1, 1904  |
| 1,254,264    | Oeschger     | ----- | Jan. 22, 1918 |
| 1,355,074    | Cleveland    | ----- | Oct. 5, 1920  |
| 45 1,529,168 | Cleveland    | ----- | Mar. 10, 1925 |
| 1,696,036    | Heinzman     | ----- | Dec. 18, 1928 |
| 1,761,186    | Baker        | ----- | June 3, 1930  |
| 1,837,159    | Fellows      | ----- | Dec. 15, 1931 |
| 1,949,713    | Gravell      | ----- | Mar. 6, 1934  |
| 50 2,203,063 | Schueler     | ----- | June 4, 1940  |
| 2,228,836    | MacQuaid     | ----- | Jan. 14, 1941 |
| 2,254,980    | Simmons      | ----- | Sept. 2, 1941 |
| 2,255,493    | Pfalzgraff   | ----- | Sept. 9, 1941 |
| 55 2,334,177 | Dishauzi     | ----- | Nov. 16, 1943 |
| 2,479,423    | Snyder       | ----- | Aug. 16, 1949 |
| 2,516,008    | Lum          | ----- | July 18, 1950 |
| 2,516,685    | Douty et al. | ----- | July 25, 1950 |
| 2,529,762    | Brisse       | ----- | Nov. 14, 1950 |

FOREIGN PATENTS

|            |               |       |               |
|------------|---------------|-------|---------------|
| 60 673,638 | Great Britain | ----- | June 11, 1952 |
|------------|---------------|-------|---------------|